

June 15, 1954

P. KÜMMEL

MELT SPINNING METHOD

2,681,266

Filed Aug. 11, 1950



INVENTOR.  
PAUL KÜMMEL

BY

*Frank E. Murphy*

ATTORNEY

## UNITED STATES PATENT OFFICE

2,681,266

## MELT SPINNING METHOD

Paul Kümmel, Ems, Switzerland, assignor to  
 Inventa A. G. für Forschung und Patentver-  
 wertung, Lucerne, Switzerland

Application August 11, 1950, Serial No. 178,788

1 Claim. (Cl. 18—54)

**1** This invention relates to an improved method for molten flux spinning of polyamides.

More particularly the invention relates to a new method for molten flux spinning of poly- $\epsilon$ -aminocaprolactam.

In the usual apparatus for molten spinning of polyamides, the polyamide is molten in a melting device, flows from there into a supply chamber (sump) and goes from there, via a pressure pump and a measuring pump to the spinning nozzle.

The entire device is surrounded by a heating jacket which heats the spinning mass to spinning temperature, i. e. to at least 40° C. above the melting point of the polyamide. In order to achieve this, the temperature of the heating jacket must lie 20—30° C. higher, or, in all, 60—70° C. above the melting point of the polyamides, and the same temperature obtains in the melting device.

This kind of spinning apparatus is unsuited to the spinning of polycaprolactam. If the polymer of the caprolactam is spun in such an apparatus, the silk has an extract content of 5.9% monomers when starting with a polyamide containing 1% extract (with a pump output of 12 g./min. and a sump of 550 ccm.). Such a high extract content is not bearable for the production of fibers and threads; the monomers must be subsequently washed out and are lost in the wash-water.

It has been found that the reversion of monomers in the polyamide flux can be considerably reduced by heating the flux to a temperature only just above the melting point of the polymerisate and raising it to the necessary temperature only immediately before spinning.

In the process according to the invention, the melting device and the supply chamber (sump) are provided with separate heating jackets whose temperature lies just above the melting point of the polymerisate.

It is necessary to make the sump larger than hitherto usual, so that the molten supply contained therein will be sufficient for spinning about 90 minutes, as only thus will the polymerisate be completely liquified at the low melting temperature.

The accompanying drawing shows schematically a spinning device for molten flux spinning according to the invention. Reference No. 1 is the heating jacket for the melting-device 2 as well as the supply chamber (sump) 3 for the flux supplied by the melting-device 2.

In the process according to the invention, the

**2** flux, at a temperature of 225° C. flows into block 4, heated by the heating jacket 5 via the pump 6 to the nozzle 7, whereby this spinning device proper is heated as high as required by the spinning process.

The following test data explain the process in accordance with the invention:

The sump volume permits 90 minutes of spinning time, i. e. the time of sojourn in the sump amounts to 90 minutes. The material to be molten consists of poly- $\epsilon$ -aminocaprolactam in the form of lengths or flakes of suitable size, from which the monomer has been extracted and which contains preferably not more than 1% water-soluble monomers. The temperature of devices 1 and 2 and thus of the melting-device 3 is 225° C. In 90 minutes the extract content increases to 1.5% as a result of thermic reversion. During the flow of the flux to the pump and from there to the nozzle there results, due to the heating of the flux to spinning temperature, which is about 250° C., a further thermic reversion of 0.5%.

The process according to the invention, with a spinning extract of 3% as compared with the 5.9% of previous processes, exhibits the important advantage of a smaller reversion of water-soluble monomers of 2.9%, which, in the hitherto practiced processes are lost with the wash-water.

**I claim:**

**1** A method of spinning poly- $\epsilon$ -amino caprolactam which comprises the steps of melting poly- $\epsilon$ -amino caprolactam flakes containing substantially not more than 1 per cent of water-soluble monomers at a temperature just above the melting point, accumulating said melt to a volume sufficient for a spinning operation of at least about 90 minutes, maintaining the accumulating melt at a temperature not exceeding about 225° C. so as to obtain a minimum of reversion to the monomer, and feeding the molten material to a spinning zone maintained at a higher temperature of about 250° C.

## References Cited in the file of this patent

## UNITED STATES PATENTS

| Number    | Name           | Date          |
|-----------|----------------|---------------|
| 2,207,426 | Bailey         | July 9, 1940  |
| 2,217,743 | Greenewalt     | Oct. 15, 1940 |
| 2,241,321 | Schlack        | May 6, 1941   |
| 2,514,189 | Spencer et al. | July 4, 1950  |
| 2,515,136 | Pigott         | July 11, 1950 |